

# United States Patent [19]

Snape

[11] 3,811,872

[45] May 21, 1974

[54] **CORROSION RESISTANT HIGH STRENGTH ALLOY**

[75] Inventor: **Edwin Snape, Monsey, N.Y.**

[73] Assignee: **The International Nickel Company, Inc., New York, N.Y.**

[22] Filed: **Apr. 21, 1971**

[21] Appl. No.: **136,217**

[52] U.S. Cl. .... **75/122, 75/128 W, 75/128 B, 75/171**

[51] Int. Cl. .... **C22c 39/00, C22c 19/00**

[58] Field of Search .... **75/128 B, 128 R, 122, 171**

[56] **References Cited**

UNITED STATES PATENTS

|           |        |                 |          |
|-----------|--------|-----------------|----------|
| 2,536,033 | 1/1951 | Clarke .....    | 75/125   |
| 2,981,621 | 4/1961 | Thielmann ..... | 75/171 H |
| 3,034,286 | 5/1962 | Bourquin .....  | 75/171 H |

|           |         |                     |          |
|-----------|---------|---------------------|----------|
| 3,068,096 | 12/1962 | Elbaum .....        | 75/171 H |
| 3,251,683 | 5/1966  | Hammond .....       | 75/128 B |
| 3,360,363 | 12/1967 | Herchenroeder ..... | 75/128 R |
| 3,519,419 | 7/1970  | Gibson .....        | 75/128 R |
| 3,532,491 | 10/1970 | Floreen .....       | 75/128 B |
| 3,547,625 | 12/1970 | Bieber .....        | 75/128 B |

Primary Examiner—Hyland Bizot

Attorney, Agent, or Firm—Raymond J. Kenny; Ewan C. MacQueen

[57] **ABSTRACT**

A high strength corrosion resistant steel containing correlated amounts of iron, chromium, molybdenum, cobalt, nickel, carbon and other constituents such as aluminum and titanium. The alloys resist pitting and crevice corrosion as well as general corrosion and are capable of offering tensile strengths well above 150,000 psi.

14 Claims, No Drawings

## CORROSION RESISTANT HIGH STRENGTH ALLOY

As is known in the metallurgical art, there are a number of alloys commercially available which might be characterized, relatively speaking, as "highly corrosion resistant", many of the stainless steels and certain nickel and copper-base alloys being illustrative. And, there are any number of alloys which upon hardening manifest "high tensile strength", the low alloy and martensitic steels being rather exemplary. Considerably less in number, however, are those alloys capable of delivering a combination of both properties together with good workability, adequate ductility, etc.

When consideration is given to the extreme aggressiveness of various corrosive media, the situation becomes somewhat more acute. For example, the austenitic stainless steels, their numerous attributes notwithstanding, seemingly manifest a propensity to undergo premature failure in stagnant seawater and other various oxidizing chloride solutions, e.g., ferric chloride. But, the demand for more corrosion resistant materials in such environments is more than likely to persist, as would appear evident from the increased activity in such rapidly developing areas such as desalination, undersea mining, oceanography in general, etc.

When tensile strength requirements on the order of, say, 150,000 to 275,000 psi together with good fabricability, ductility, etc., are injected into the picture, it becomes more readily apparent as to why so very few alloys are commercially available capable of operating satisfactorily under such conditions. It is to this overall problem to which the present invention is primarily, though by no means singularly, addressed.

In any case, it has been found that certain hardened alloys containing correlated percentages of iron, nickel, cobalt, chromium, molybdenum, etc., offer exceptional combinations of corrosion resistance and tensile strength together with good fabricability and adequate ductility.

Generally speaking, the present invention contemplates highly corrosion resistant, work hardenable alloys capable of developing a special microstructure and high strength as more fully herein described, the alloys containing (in weight per cent) from 5 to 30 percent chromium, about 2 to 15 percent molybdenum with the total percentage of molybdenum plus chromium being from about 20 to about 35 percent, about 10 to 30 percent nickel, about 13 to 30 percent cobalt, the ratio of nickel to cobalt not exceeding about 1.5:1, up to 0.15 percent, but most beneficially not more than 0.05 or 0.03 percent, carbon, up to about 3 percent titanium, up to about 3 percent aluminum and the balance essentially iron, the iron preferably constituting at least about 15 or 20 percent but not less than 10 percent of the alloys.

In addition to the above chemistry and in order to achieve tensile strength levels as set forth herein, the steels should be characterized by a microstructure comprised essentially of a face-centered cubic (austenitic) matrix throughout which epsilon or a phase closely resembling epsilon and consisting of platelets are substantially and relatively uniformly dispersed, the platelets being present in at least a small but effective amount, e.g., at least about 2 or 3 percent by volume, sufficient to impart enhanced tensile strength to the matrix. Most advantageously, these platelets formed in and distributed throughout the austenite, are present in an amount of at least 5 percent by volume, a volume of

about 7.5 to 20 percent being quite satisfactory, although up to 45 percent can be present.

In carrying the invention into practice, the sum of the molybdenum plus chromium should not exceed about 35 percent; otherwise, hot working is at best unnecessarily rendered more difficult, due, it is believed, to the tendency of these constituents to form sigma, an embrittling phase which can promote the onset of cracking. For this and other reasons, it is preferred that the total percentage of molybdenum plus chromium not exceed about 30 percent; however, at least 20 percent thereof is required for good corrosion resistance. In striving for the optimum by way of resistance to crevice and pitting corrosion in particular, the chromium should be from 16 to 30 percent, the molybdenum should be from 2 to 10 percent and these components should be correlated such that the total sum of three-fourths the percentage of chromium plus the percentage of molybdenum is at least about 18 percent and is beneficially at least about 20 percent.

It is also noteworthy to point out that it has been determined that molybdenum confers improved tensile ductility and also increases the work hardening rate, particularly at reductions of at least 25 percent, e.g., 40 percent, or more. Accordingly, it is preferred that the molybdenum be not less than 4 percent.

With regard to cobalt, it exercises a potent influence in bringing about the formation in the austenite of the epsilon-like platelets by virtue of which the high strength levels characteristic of the subject alloys are in large part achieved. Oddly enough, given the voluminous information available concerning the mechanisms by which alloy matrices are conventionally hardened, e.g., age hardening (including precipitation hardening), cold working, refrigeration, matrix stiffening, combinations thereof, etc., in marked contrast scant attention ostensibly has been accorded the type of strengthening described herein. This might possibly stem from embrittlement considerations. Regardless of the reasons, I am presently aware of but one instance in which this phenomenon has been advanced commercially. This occurred in respect of a relatively high cobalt-nickel-base alloy, an alloy which appears, at best, to be difficultly fabricable as well as costly.

Preliminary metallographic examination of various alloys indicated the thin parallel platelets to be of the epsilon phase; however, using electron transmission microscopy and electron diffraction the platelets appeared to be more on the order of "deformation twins". It is deemed that this holds true for alloys within the invention up to about 25 percent cobalt. At the higher cobalt percentages, e.g., 28-30 percent, it is considered that epsilon is likely present although it might be difficult to resolve. As is known, deformation twins and the epsilon phase are quite difficult to differentiate. In any case and irrespective of terminology, the thin parallel platelets are formed by cold working alloy compositions within the invention.

The percentage of cobalt need not exceed about 21 or 22 percent since it has been found that higher amounts do not appreciably increase work hardening rate. Thus, it is deemed about 15 percent to 23 or 25 percent cobalt is extremely effective in providing steels at the higher order of tensile strength without adversely affecting other characteristics. Above about 30 percent cobalt, improvement is not sufficiently great to warrant the added cost. Percentages below 13 percent and down to 10 percent can be used but a correlation between nickel and cobalt should be maintained such that

the ratio of nickel to cobalt does not exceed about 1.2:1.

Nickel is particularly useful in precluding formation of unwanted martensite during cold working. It is thought excessive martensite can contribute to or impart a condition of embrittlement. A nickel range of 15 percent to 23 or 25 percent is quite beneficial and a combined nickel plus cobalt content of not greater than 45 or 50 percent is satisfactory from a technological viewpoint and is economically attractive commercially.

Tensile strengths of the alloys can be increased through the incorporation of aluminum and/or titanium. Up to 3 percent each can be present but higher amounts should be avoided to obviate hot working difficulties. A range of 0.05 percent or 0.1 to 2 percent of either or both can be used, although a combined percentage of not more than 3 percent is much preferred. A small amount of titanium, e.g., from 0.05 percent to 0.3 or 0.5 percent is beneficial for good forgeability and also can provide improved corrosion resistance.

With regard to such elements as silicon, manganese and carbon, while up to 2.5 percent silicon can be added to the subject alloys, particularly in castings, it can detract from corrosion resistance and promote edge cracking during hot working if found in amounts of, say, 1.5 or 2 percent or more in the presence of molybdenum above about 7 or 8 percent or a high combined percentage of chromium plus molybdenum, say, much above 25 or 26 percent, e.g., 28 percent or more. Such alloys are not recommended and, thus, the percentage of any silicon need not exceed 0.5 or 1 percent. Nor does manganese have to exceed 1 to 1.5 percent and it is preferred that it be below about 0.8 percent. Because of its potential effect on corrosion resistance and carbide formation, carbon should not be found in percentages above about 0.05 percent, a range of from trace amounts to 0.03 or 0.04 percent being preferred.

A particularly advantageous alloy composition in accordance herewith is as follows: about 10 to 28 percent chromium, about 5 to about 10 percent molybdenum, the sum of the chromium plus molybdenum being from 24 to 30 percent, about 15 to 25 percent nickel, about 15 to 25 percent cobalt, carbon in an amount up to 0.05 percent, up to 2 percent titanium, up to 2 percent aluminum, up to 1 percent silicon, up to 1 percent, e.g., about 0.2 to 0.8 percent, manganese and the balance essentially iron, the iron preferably constituting at least 20 or 25 percent of the alloy.

In order to give those skilled in the art a better appreciation of the invention, the following illustrative data are given.

Using vacuum induction melting and high purity materials (electrolytic iron, cobalt and nickel, vacuum grade chromium, molybdenum pellets, etc.) a series of alloys were prepared, the compositions being given in Table I.

TABLE I

| Alloy | C, % | Si, % | Mn, % | Ni, % | Cr, % | Co, % | Mo, % | Ti, % | Al, % | Fe, % |
|-------|------|-------|-------|-------|-------|-------|-------|-------|-------|-------|
| 1     | .033 | 2.05  | .59   | 15.1  | 21.6  | 24.2  | 4.8   | 0.1   | n.a.  | Bal.  |
| 2     | .029 | 1.98  | .55   | 19.2  | 21.6  | 19.7  | 5.9   | 0.1   | n.a.  | Bal.  |
| 3     | .026 | .33   | .50   | 15.6  | 11.4  | 20.4  | 10.0  | n.a.  | .05   | Bal.  |
| 4     | .024 | .37   | .48   | 14.8  | 10.4  | 19.9  | 9.9   | 1.9   | .08   | Bal.  |
| 5     | .026 | .33   | .51   | 15.2  | 11.1  | 20.3  | 10.1  | n.a.  | .08   | Bal.  |
| 6     | .044 | .40   | .35   | 18.6  | 21.3  | 19.0  | 3.9   | n.a.  | -     | Bal.  |
| 7     | .031 | .31   | .21   | 18.6  | 19.0  | 19.7  | 7.0   | n.a.  | -     | Bal.  |
| 8     | .022 | .46   | .20   | 19.2  | 18.8  | 20.1  | 9.7   | n.a.  | -     | Bal.  |
| 9     | .019 | .12   | .64   | 21.4  | 18.8  | 21.5  | 7.0   | 1.74  | -     | Bal.  |

n.a. = none added, not analyzed

In producing the alloys, the nickel, cobalt, iron and molybdenum were charged, heated to about 2850°F and, for Alloys 6-9, held thereat, for about 5 minutes for a carbon boil, the chromium, silicon and, if any, titanium and aluminum then being added. Alloys 1-5 were deoxidized with calcium-silicon and nickel-magnesium. Pouring was conducted at about 2,800°F and the resulting ingots (30 lb.) were soaked 2 hours at 2,200°F with half of each ingot being rolled at about 2,150°F to  $\frac{1}{4}$ -inch plate, the other half being rolled to  $\frac{1}{2}$ -inch round bar. Upon solution treating at about 2,200°F, for 1 hour, followed by water quenching, the  $\frac{1}{2}$ -inch bars were cold drawn in an amount indicated in Table II to induce formation of the platelets in the austenite. Tensile and elongation properties are also reported in Table II.

TABLE II

| Alloy No. | Cold Reduction, % | U.T.S., psi | Y.S., psi | El., % |
|-----------|-------------------|-------------|-----------|--------|
| 20        | 1                 | 224,200     | 173,500   | 16     |
|           | 2                 | 210,800     | 181,700   | 16     |
|           | 3                 | 206,600     | 185,600   | 11     |
|           |                   | 241,600     | 236,000   | 4      |
|           | 4                 | 206,600     | 190,800   | 9      |
|           |                   | 214,400     | 187,400   | 5      |
|           | 5                 | 198,700     | 185,400   | 8      |
|           |                   | 206,900     | 183,800   | 6      |
|           | 6                 | 194,500     | 176,300   | 11.5   |
|           |                   | 241,300     | 214,000   | 3.5    |
| 30        | 7                 | 205,800     | 190,800   | 14     |
|           | 8                 | 253,000     | 215,400   | 5      |
|           |                   | 228,600     | 207,500   | 12     |
|           | 9                 | 275,000     | 232,100   | 2.5    |
|           |                   | 209,200     | 183,200   | 10.5   |
|           | 80                | 245,200     | 212,300   | 9      |

As reflected by the data in Table II, tensile strengths well above 200,000 psi were attained together with good ductility. Charpy V-notch results were determined for Alloys 1 and 2 and the values were 25.5 and 21 ft. lbs., respectively.

Alloys 3, 4 and 5 were, subsequent to being cold worked, also aged at 900°F. for about 3 hours and the results are given in Table III.

TABLE III

| Alloy No. | Cold Reduction, % | U.T.S., psi | Y.S., psi | El., % |
|-----------|-------------------|-------------|-----------|--------|
| 50        | 3                 | 226,900     | 213,600   | 9      |
|           | 85                | 263,400     | 238,300   | 5      |
|           |                   | 241,500     | 227,900   | 9      |
|           | 85                | 257,500     | 253,300   | 5      |
|           |                   | 223,500     | 212,500   | 7      |
|           | 85                | 245,200     | 237,500   | 3      |

Although alloys of Table I were vacuum melted, air melting procedures can also be used to marked advantage. In this connection, a 100 lb. heat (Alloy 10) was produced by air melting practice and thereafter tested in much the same manner as the alloys of Table I. This particular alloy nominally contained 0.03 percent carbon, 0.4 percent silicon, 0.4 percent manganese, 25 percent nickel, 20 percent chromium, 20 percent cobalt, 8.5 percent molybdenum, balance essentially iron and usual impurities. Deoxidation was accomplished with calcium-silicon and nickel-magnesium. It was hot rolled at an initial temperature of about 2,100°F, solution treated at 2,100-2,200°F and quenched prior to cold rolling. After being cold worked 78 percent and then aged at 900°F for 3 hours, the following test results were obtained: an ultimate tensile strength of 260,000 psi, a 0.2 percent yield strength of 250,000 psi, an elongation of 9 percent, a reduction in area of 42 percent, an Rc hardness of 49 and a notched tensile to ultimate tensile ratio of 1.2:1. Elevated temperature properties were also quite good.

In Table IV are set forth the results of a ferric chloride corrosion test which involved exposing cold worked and/or cold worked and aged specimens having a surface area of about 1 square inch in a 10 percent ferric chloride solution for a period of 72 hours. Compositions are also given in Table IV. Crevices were intentionally formed by wrapping a  $\frac{1}{4}$ -inch rubber band about the specimens. As will be appreciated by those skilled in the art, this overall test is one of an extremely aggressive nature. The results given represent the overall weight loss in milligrams determined with regard to the entire specimen surface area.

TABLE IV

| Alloy | C, % | Si, % | Mn, % | Ni, % | Cr, % | Co, % | Mo, % | Ti, % | Wt. Loss,<br>Cold<br>Rolled | Wt. Loss,<br>Aged |
|-------|------|-------|-------|-------|-------|-------|-------|-------|-----------------------------|-------------------|
| 10    | .048 | .51   | .22   | 19.9  | 20.5  | 20.3  | 8.2   | .43   | nil                         | nil               |
| 11    | .034 | .50   | .19   | 25.1  | 20.5  | 20.2  | 8.3   | .44   | nil                         | nil               |
| 12*   | .024 | .50   | .27   | 20.4  | 20.2  | 20.1  | 8.5   | .27   | nil                         | nil               |
| 13*   | .022 | .47   | .23   | 25.4  | 20.0  | 20.4  | 8.5   | .25   | nil                         | nil               |

\* air melted; otherwise, vacuum melted.

nil = less than 1 mg.

With further regard to the above ferric chloride test, none of the specimens exhibited (upon visual examination) any evidence of pitting or crevice corrosion. As to other corrosive media, alloys within the invention manifested a high degree of resistance to 10%  $H_2SO_4$  and also to 10% HCl in 7 day tests.

The above corrosion data are indicative of the excellent corrosion behavior characteristic of alloys within the invention. It might also be added that potentiostatic polarization tests conducted to date confirm that the alloys offer marked resistance to corrosion, the alloys displaying an ability to be readily passivated, particularly at the higher molybdenum levels.

As indicated above, alloys in accordance herewith can be prepared by either vacuum processing, including vacuum refining, or by air melting techniques. To date, in some instances ductility has been slightly better with vacuum melted materials particularly with cold reductions greater than 90 percent. While air melted alloys have been cold drawn 99 percent in the production of wire, vacuum melted alloys have been successfully cold drawn approximately 99.7 percent while re-

taining sufficient ductility to pass the "kink" and "wrap" tests. Formation of the platelets in the austenite is, as indicated herein accomplished most conveniently by cold working at about room temperature.

5 Alloys contemplated within the invention are useful as fasteners particularly in marine environments. Other marine hardware would include parts for pumps, valves, shafting, shocks, cleats, wrought fittings, etc. The alloys can also be used in chemical plant equipment and for such diverse utility as aerospace applications. Also, the alloys can be produced and used in various conventional mill forms including sheet, strip, bar, rod and also as suggested above in the form of high strength wire.

15 In referring to the iron content of the alloys as constituting the "balance" or "balance essentially", it is to be understood, as will be appreciated by those skilled in the art, that the presence of other elements is not excluded, such as those commonly present as incidental elements, e.g., deoxidizing and cleansing constituents, and impurities normally associated therewith in small amounts that do not adversely affect the basic characteristics of the alloys. Non essential elements that can be present include up to 2 percent each of copper and zirconium, up to 0.05 percent boron and up to 0.05 percent selenium.

20 25 30 Although the present invention has been described in conjunction with preferred embodiments, it is to be understood that modifications and variations may be resorted to without departing from the spirit and scope of the invention, as those skilled in the art will readily understand. Such modifications and variations are consid-

ered to be within the purview and scope of the invention and appended claims.

I claim:

50 1. A corrosion resistant alloy having high strength and characterized by a microstructure comprised essentially of a face-centered cubic matrix throughout which platelets are substantially and relatively uniformly dispersed, the platelets being present as a result of cold working the alloy and being present at least in a small but effective amount sufficient to impart enhanced tensile strength to the matrix, said alloy consisting essentially of from 5 to 30 percent chromium, from 2 to 15 percent molybdenum with the proviso that the total percentage of molybdenum plus chromium be from about 20 to about 35 percent, about 10 to 30 percent nickel, about 10 to 30 percent cobalt with the further provisos that when the cobalt content is less than about 13 percent the ratio of nickel to cobalt does not exceed about 1.2:1 and when the cobalt is 13 percent more the said ratio does not exceed 1.5:1, up to about 0.15 percent carbon, up to about 3 percent titanium, up to about 3 percent aluminum and the balance essen-

tially iron, the iron constituting at least 10 percent of the alloy.

2. An alloy in accordance with claim 1 containing at least about 13 percent cobalt and at least about 15 percent iron and in which the carbon does not exceed about 0.05 percent and in which the platelets are present in an amount of at least 5 percent by volume.

3. An alloy in accordance with claim 2 in which the platelets are present from about 5 to 45 percent by volume.

4. An alloy in accordance with claim 2 in which the sum of chromium plus molybdenum does not exceed 30 percent.

5. An alloy in accordance with claim 4 in which iron is present in an amount of at least 20 percent.

6. An alloy in accordance with claim 2 in which the carbon content does not exceed 0.03 percent.

7. An alloy in accordance with claim 2 which contains at least one constituent from the group consisting of titanium and aluminum in an amount of at least 0.05 percent.

8. An alloy in accordance with claim 7 which contains 0.05 to 3 percent of aluminum plus titanium.

9. An alloy in accordance with claim 2 in which the molybdenum content is at least 4 percent.

10. An alloy in accordance with claim 2 in which the chromium is from 16 to 30 percent, the molybdenum is from 2 to 10 percent and the total sum of three-

fourths the percentage of chromium plus the percentage of molybdenum is at least 20 percent.

11. An alloy in accordance with claim 2 in which any manganese or silicon does not exceed about 1 percent, respectively.

12. An alloy in accordance with claim 2 consisting essentially of about 10 to 28 percent chromium, 5 to 10 percent molybdenum, about 15 to 25 percent nickel, about 15 to 23 percent cobalt, about 0.001 to 0.05 percent carbon, up to 2 percent titanium, up to 2 percent aluminum, up to 1 percent silicon, and up to about 0.8 percent manganese.

13. An alloy in accordance with claim 12 containing at least 0.2 percent manganese.

14. A ductile, workable, corrosion resistant alloy possessing a high degree of resistance to oxidizing chloride media such as stagnant seawater and adapted to afford high tensile strength and consisting essentially of from 5 to 30 percent chromium, about 2 to 15 percent molybdenum with the proviso that the total percentage of molybdenum plus chromium be from about 20 to about 30 percent, about 10 to 25 percent nickel, about 15 to 23 percent cobalt, with the further proviso that the ratio of nickel to cobalt does not exceed 1.5:1, up to about 0.15 percent carbon, up to about 3 percent titanium, up to about 3 percent aluminum and the balance essentially iron, the iron constituting at least 20 percent of the alloy.

\* \* \* \* \*

30

35

40

45

50

55

60

65